

## UNITED STATES PATENT OFFICE

2,203,493

## TREATMENT OF CELLULOSIC MATERIAL

John Gwynant Evans, Henry Alfred Piggott, Reginald John William Reynolds, John Donald Rose, and Eric Everard Walker, Blackley, Manchester, England, assignors to Imperial Chemical Industries Limited, a corporation of Great Britain

No Drawing. Application June 23, 1938, Serial No. 215,495. In Great Britain June 30, 1937

6 Claims. (Cl. 8—120)

The present invention relates to a process of treatment of cellulosic material whereby it is rendered capable of being dyed with acid wool dyestuffs or acid chrome dyestuffs, the dyeings so obtained being fast to washing or other aqueous treatments.

By cellulosic material we mean any material consisting of or containing natural cellulose fibre such as cotton, linen or jute, or regenerated cellulose fibre or filament, either spun, woven or in the form of paper or cardboard; we include also regenerated cellulose in the form of film.

It is an object of the invention to make it possible to dye cellulosic materials with the classes of dyestuffs known as acid wool dyestuffs and acid chrome dyestuffs. As is known, these are characterised by the presence of sulphonic and/or carboxylic acid groups. Other dyestuffs are known, equally capable of dyeing wool. These contain other acid groups, e. g., the sulphuric ester group. These also are regarded as acid wool dyestuffs for the purposes of this invention.

The invention is particularly adapted to the dyeing of regenerated cellulose as by its means that fibre can be given affinity for acid dyestuffs. Thus the dyeing of viscose staple fibre materials, especially mixed fibres and union yarns of viscose staple fibre and wool, is facilitated.

The invention comprises the application to cellulosic material of a compound in the molecule of which there is at least one of each of two kinds of functional groups. These two functional groups are (A) an ammonium or similar group capable of so interacting during dyeing with a dyestuff of the kind described so that, as is supposed, the material carries or encloses within its intermicellar or other interstices pigmentary substance which can be regarded as an organic salt of the dyestuff acid; and (B) a group originally such that the compound is water soluble but so adapted to self or conjoint reaction on application of heat that the heating treatment referred to results in the fixation on the material of a substance no longer containing group (B) but still containing group (A).

More particularly group (B) is such that it is capable of reacting with formaldehyde. Suitable groups classified under (B) are such that the compound is a carboxylic amide, a substituted urea or a carbamate.

In these compounds the functional groups (A) and (B) may be linked together by arylene or alkylene radicals which may provide the entire link, or may be part of a link, e. g., alkylene

links may themselves be linked by oxygen or nitrogen atoms.

According to the invention cellulosic material is treated at a relatively low temperature with a solution of a compound constituted as described when necessary in the presence of or subsequently with formaldehyde or a substance capable of yielding formaldehyde in the conditions of reaction, and is then heated for a short time to a moderately elevated temperature.

As compounds coming under the above description as containing the groups (A) and (B) there spoken of, there come to be mentioned those of the general formula



15

wherein the symbols used, so far as they do not carry their known and customary significance, are explained below.

$R'$  stands for hydrogen or an alkyl, aralkyl or aryl radical and  $R''$  and  $R'''$  stand for the same or different alkyl or aryl radicals; or  $R'R''N$  taken by itself may stand for a tertiary amine, which is a heterocyclic compound, typified by pyridine of the one class, or the alkyl piperidines of another; or  $R''R'''NH$  taken by itself may stand for a heterocyclic secondary amine, e. g. piperidine.

$L$  stands for the link spoken of above, i. e., it stands for a divalent organic radical, for instance:



35

$X$  stands for an acid radical.

Compounds suitable to be used in the process of the invention may conveniently be made by the processes described in British Patents Nos. 497,043; 497,368, and 497,485.

It is a further feature of the invention to use, instead of the compounds represented by the general formulae given above the suitable products of their condensation with formaldehyde, for example, their methylol derivatives. As will be seen, here a preformed formaldehyde compound is used, but the treatment may nevertheless be carried out in presence of a further quantity of formaldehyde or formaldehyde yielding substance.

As suitable formaldehyde yielding substances there may be mentioned, for example, dimethylol urea, the dimethyl ether of dimethylol urea and methylol urethane.

55

The invention is carried into practical effect in a number of ways. Thus (a) the cellulosic material is impregnated with a solution, for example, an aqueous solution of one of the compounds mentioned, the solution containing also formaldehyde or a formaldehyde yielding substance. The impregnated material is then dried and subjected to a short heat treatment. If desired, the drying and heating treatment may be carried out in one step.

(b) The cellulosic material is impregnated with a solution of one or more of the said compounds and exposed in the wet or dry state to formaldehyde vapour at atmospheric or higher pressure, preferably at elevated temperature.

(c) The cellulosic material is impregnated with a solution of one or more of the compounds mentioned, then, preferably after drying, is treated in a bath containing formaldehyde or a formaldehyde yielding substance, dried, and finally subjected to a short heat treatment. Again if necessary, the drying and heat treatment may be carried out as one step.

(d) When using pre-formed condensation products, such as the methylol compounds mentioned, the treatment is carried out by any of the foregoing methods, or the simultaneous or subsequent treatment with formaldehyde or a formaldehyde-yielding substance may be omitted, as already explained.

The impregnation mentioned may be carried out with advantage by use of an acidified liquor containing e. g., boric acid, acetic acid, tartaric acid, lactic acid, tannic acid or an acid substance or compound which yields acid under the conditions of drying or heating, e. g., ammonium dihydrogen phosphate, ammonium chloride, ammonium thiocyanate or sodium bisulphite. The heat-treatment may also be carried out in acid conditions by application of acid as vapour or in other ways.

The heat treatment above referred to may be for a short period, for example, 5 to 30 minutes, at a temperature of 100°-140° C. Alternatively it may be provided by steaming the treated material for a short time, for example, ½ to 1 hour.

The invention is illustrated but not limited by the following examples, in which the parts are by weight.

#### Example 1

Finely woven cotton material of the kind known as limbric is impregnated at room temperature with a solution containing 2 parts of the condensation product of formaldehyde and  $\beta$ -ureidoethylpyridinium chloride of the formula



and 0.3 part of ammonium dihydrogen phosphate in 98 parts of water. The material is squeezed to remove excess of liquor and is then dried rapidly in a current of warm air at a temperature of 60° C. The dry fabric is heated for 5 minutes at a temperature of 120° C. After heating the fabric is well rinsed in warm water. The material may now be dyed with acid wool colours.

For example, 100 parts of treated cotton is rinsed in water and entered at 40°-50° C. into 20 times its weight of a solution containing 1 part of Azo Geranine 2G (Colour Index No. 31) in 1000 parts of water. The dyebath is raised to the boil and maintained at the boil for 30 minutes. The material is then removed, rinsed and dried. The dye is almost completely exhausted from the dyebath, the treated material being dyed to a

full red shade. The dyeing shows good resistance to water and to washing treatments.

Alternatively, 100 parts of the treated cotton may be dyed in a bath containing 1 part of Coomassie Violet 2R (Colour Index No. 758), 3 parts of acetic acid and 10 parts of sodium sulphate in 3000 parts of water, using the dyeing conditions described above. The material is thus dyed to a full violet shade which has good resistance to water and to soap washing.

#### Example 2

Viscose rayon fabric is soaked in a solution containing 2 parts of ureidoethylpyridinium chloride of the formula



0.3 part of ammonium dihydrogen phosphate and 3.0 parts of a 40% aqueous solution of formaldehyde in 100 parts of cold water. The material is squeezed until it contains its own weight of solution and is dried in a current of hot air at 60° C. It is then heated for ½ hour at 140° C. The material now has enhanced affinity for acid wool dyestuffs. It may be dyed, for example with Coomassie Violet 2R (Colour Index No. 758) by the method described in the previous example.

#### Example 3

Viscose rayon stockinette is soaked in a solution containing 2 parts of carbamylmethylpyridinium chloride of the formula



0.3 part of ammonium dihydrogen phosphate and 12.5 parts of a 40% aqueous formaldehyde solution in 100 parts of cold water. The material is squeezed until it contains its own weight of the solution and is dried in a current of hot air at 60° C. It is then heated for ½ hour at 140° C. The material now has affinity for acid wool dyestuffs and acid chrome dyestuffs and may be dyed therewith in the manner normally used for wool dyeing. Moreover the dyeings so obtained are fast to washing and other aqueous treatments.

For example, 100 parts of viscose rayon stockinette treated as described with either of the above agents may be dyed for 1 hour at the boil in a solution containing 2 parts of Azo Geranine 2G (Colour Index No. 31), 3 parts of concentrated sulphuric acid and 10 parts of sodium sulphate in 3000 parts of water. There is thus produced a full red shade which is very fast to aqueous soap washing treatments.

If, in the above process, instead of the carbamylmethylpyridinium chloride, there is used an equal weight of p-dimethylaminophenylurea methosulphate of formula



If viscose fabric impregnated as described with either of the above agents, instead of being heated for ½ hour at 140° C., is steamed at atmospheric or slightly increased pressure for ½ hour, there is obtained a material having similarly enhanced affinity for acid wool dyestuffs.

#### Example 4

Viscose rayon fabric is soaked in a solution containing 2 parts of hydroxymethylcarbamylmethylpyridinium chloride of the formula



in 100 parts of water and is then squeezed so that

it retains its own weight of the solution. It is then heated, without previous drying, to 140° C. for 1/2 hour. The material now has affinity for acid wool dyestuffs and can be dyed therewith in the manner normally used for wool dyeing.

Thus, for example, 100 parts of the treated viscose are dyed for 1 hour at the boil in a bath containing 2 parts of Tartrazine N (Colour Index No. 640), 3 parts of concentrated sulphuric acid, 10 parts of sodium sulphate and 3000 parts of water. The dyeing so obtained has a full yellow shade which is fast to aqueous soap washing.

*Example 5*

Viscose staple fibre is soaked in a solution containing 2 parts of carbamylmethylpyridinium chloride, 0.3 part of ammonium dihydrogen phosphate and 12.5 parts of a 40% aqueous formaldehyde solution in 100 parts of water. The fibre is squeezed so that it contains its own weight of the solution and is then dried in a current of hot air at 60° C. Finally, it is heated for 1/2 hour at 140° C. The fibre now has affinity for acid wool colours and acid chrome colours and may be dyed therewith by the methods normally used for dyeing wool.

Thus, for example, 100 parts of the treated viscose fibre are dyed for 1 hour at the boil in a bath containing 2 parts of Naphthalene Orange G (Colour Index No. 151), 3 parts of concentrated sulphuric acid, 10 parts of sodium sulphate and 3000 parts of water. The fibre is thus dyed to a full orange shade which is fast to aqueous soap washing treatments.

Alternatively 100 parts of the treated fibre are dyed for 1 hour at the boil in a bath containing 8 parts of Solochrome Black WDFA (Colour Index No. 203), 3 parts of 30% aqueous acetic acid, 10 parts of sodium sulphate and 3000 parts of water. 200 parts of an aqueous 1% solution of sulphuric acid are then added and the bath is maintained at the boil for a further 15 minutes. 300 parts of an aqueous 1% solution of potassium dichromate are now added and the bath is maintained at the boil for a further 1/2 hour. The fibre is then removed from the bath, rinsed and dried. It is thus dyed to a full black shade which is fast to aqueous soap washing treatments.

*Example 6*

Viscose fabric is soaked in a solution containing 2 parts of carbamylmethylpyridinium chloride, 0.3 part of ammonium dihydrogen phosphate, 3 parts of a 40% aqueous formaldehyde solution in 100 parts of water. The fabric is squeezed until it retains its own weight of the solution and is then heated for 1/2 hour at 140° C. The material

now has affinity for acid wool colours and acid chrome colours.

Thus, for example, it may be dyed for 1 hour at the boil in a bath containing 2 parts of Coomassie Navy Blue 2RN (Colour Index No. 289), 0.5 part of potassium dichromate and 3000 parts of water. The material is then rinsed and dried. It is thus dyed a deep blue shade which has good fastness to aqueous soap washing.

We claim:

1. A process for enhancing the affinity of cellulosic material for acid wool dyestuffs and acid chrome dyestuffs which comprises treating the said material with a solution of an organic compound selected from the class consisting of carboxylic amides, substituted ureas, and carbamates, said compound having the general formula  $RR'R''N(X)-L-CO-NH_2$  wherein  $RR'R''N$  as a whole represents the entire molecular structure of an amine selected from the class consisting of aliphatic secondary amines, heterocyclic secondary amines, aliphatic tertiary amines, mixed tertiary amines, and heterocyclic tertiary amines,  $X$  stands for an acid radical, and  $L$  stands for a divalent organic radical selected from the group:  $-\text{CH}_2-$ ,  $-\text{CH}_2\text{CONH}-$ ,  $-\text{CH}_2\text{CH}_2\text{NH}-$ ,  $-\text{CH}_2\text{CH}_2\text{O}-$ , and  $-\text{C}_6\text{H}_4\text{NH}-$ ; and the formaldehyde condensation products of said carboxylic amides, substituted ureas, and carbamates, and then heating the so impregnated material for a short time to a moderately elevated temperature sufficient to cause said organic compound to become fixed on the said cellulosic material.

2. A process as set forth in claim 1 wherein the impregnating solution also contains a substance selected from the class consisting of formaldehyde and formaldehyde yielding substances.

3. A process as set forth in claim 1 wherein the impregnating solution also contains a substance selected from the class consisting of acids and acid yielding substances.

4. A process as set forth in claim 1 wherein the substituted urea which is employed is beta ureidoethylpyridinium chloride.

5. A process as set forth in claim 1 wherein the substituted urea which is employed is p-di-methylaminophenylurea methosulphate.

6. A process as set forth in claim 1 wherein the carboxylic amide which is employed is carbamylmethylpyridinium chloride.

JOHN GWYNANT EVANS.

HENRY ALFRED PIGGOTT.

REGINALD JOHN WILLIAM REYNOLDS.

JOHN DONALD ROSE.

ERIC EVERARD WALKER.